



US009598797B1

(12) **United States Patent**  
**Zhu**

(10) **Patent No.:** **US 9,598,797 B1**  
(45) **Date of Patent:** **Mar. 21, 2017**

(54) **CARBON-CONTAINING ARC-RESISTANT ARAMID FABRICS FROM DISSIMILAR YARNS**

(71) Applicant: **E I DU PONT DE NEMOURS AND COMPANY**, Wilmington, DE (US)

(72) Inventor: **Reiyao Zhu**, Moseley, VA (US)

(73) Assignee: **E I DU PONT DE NEMOURS AND COMPANY**, Wilmington, DE (US)

(\*) Notice: Subject to any disclaimer, the term of this patent is extended or adjusted under 35 U.S.C. 154(b) by 0 days.

(21) Appl. No.: **15/354,208**

(22) Filed: **Nov. 17, 2016**

**Related U.S. Application Data**

(60) Provisional application No. 62/382,548, filed on Sep. 1, 2016.

(51) **Int. Cl.**

**D03D 15/12** (2006.01)

**D03D 1/00** (2006.01)

**A41D 31/00** (2006.01)

(52) **U.S. Cl.**

CPC ..... **D03D 1/0035** (2013.01); **A41D 31/0022** (2013.01); **D03D 15/12** (2013.01); **D10B 2331/021** (2013.01); **D10B 2501/04** (2013.01)

(58) **Field of Classification Search**

CPC ..... D03D 1/0035; D03D 15/12; D10B 2331/021; D10B 2501/04; A41D 31/0022

See application file for complete search history.

(56) **References Cited**

**U.S. PATENT DOCUMENTS**

3,094,511 A 6/1963 Hill et al.  
3,354,127 A 11/1967 Hill et al.

|               |         |                 |
|---------------|---------|-----------------|
| 3,673,143 A   | 6/1972  | Bair et al.     |
| 3,803,453 A   | 4/1974  | Hull            |
| 3,819,587 A   | 6/1974  | Kwoleck         |
| 3,869,429 A   | 3/1975  | Blades          |
| 4,172,938 A   | 10/1979 | Mera et al.     |
| 4,612,150 A   | 9/1986  | De Howitt       |
| 4,668,234 A   | 5/1987  | Vance et al.    |
| 4,748,065 A * | 5/1988  | Tanikella ..... |
|               |         | D06M 11/74      |
|               |         | 428/152         |
| 4,755,335 A   | 7/1988  | Ghorashi        |
| 4,883,496 A   | 11/1989 | Ghorashi        |
| 5,096,459 A   | 3/1992  | Ghorashi        |

(Continued)

**FOREIGN PATENT DOCUMENTS**

WO 0077283 A2 12/2000

**OTHER PUBLICATIONS**

Black, et al., "Fiber-Forming Aromatic Polyamides", Man-Made Fibers, Science and Technology, vol. 2, p. 297, Interscience Publishers, 1968.

*Primary Examiner* — Jeremy R Pierce

(57) **ABSTRACT**

A woven fabric suitable for use in arc protection and article of thermal protective clothing comprising the fabric, the fabric having a warp yarn dissimilar to a fill yarn, wherein a majority of the a face of the fabric is a first yarn and a majority of the opposing face of the fabric is a second yarn, wherein the second yarn comprises 25 to 100 parts aramid fiber containing 0.5 to 20 weight percent discrete homogeneously dispersed carbon particles and 0 to 75 parts aramid fiber free of discrete carbon particles; and wherein the first yarn comprises aramid fiber being free of discrete carbon particles; the fabric having a total content of 0.5 to 3 weight percent discrete carbon particles.

**12 Claims, 1 Drawing Sheet**



(56)

**References Cited**

U.S. PATENT DOCUMENTS

- 5,298,028 A \* 3/1994 Hsu ..... D01F 6/605  
8/115.6  
5,578,368 A \* 11/1996 Forsten ..... B32B 5/26  
428/902  
2009/0159149 A1 \* 6/2009 Karayianni ..... D03D 1/0088  
139/425 R  
2010/0009186 A1 \* 1/2010 Zhu ..... D02G 3/047  
428/395  
2010/0075557 A1 \* 3/2010 Shteiyer ..... D03D 1/0041  
442/203  
2012/0034835 A1 \* 2/2012 Hess ..... A41D 31/0022  
442/197

\* cited by examiner



*FIG. 1*



*FIG. 2*

## 1

CARBON-CONTAINING ARC-RESISTANT  
ARAMID FABRICS FROM DISSIMILAR  
YARNS

## BACKGROUND OF THE INVENTION

## Field of the Invention

This invention relates to fabrics and articles that provide protection to workers from electrical arcs.

## Description of Related Art

Industrial workers and others who can be exposed to electrical arcs and the like need protective clothing and articles made from thermally resistant fabrics. Any increase in the effectiveness of these protective articles or any increase in the comfort of these articles while maintaining protection performance is welcomed.

Carbon particles have been used as a spun-in pigment in the coloration of fibers, the black color of carbon being effective in generating dark shades.

It has been found that if carbon particles are spun into fibers made from fire resistant and thermally stable polymers, the resulting yarns, fabrics, and garments provide dramatically improved arc protection. However, the carbon particles tend to make fibers having a dark shade, and arc-protective fabrics and garments of lighter shade are desired in many instances. For example, garments having darker shades are more difficult to see at night and in low-visibility situations. On the other hand, some garment manufacturers simply wish to have the ability to provide a variety of color shades to address the fashion choices of their customers.

Therefore, what is needed is a method to have arc protection that is both the dramatically improved and has desirable color shades.

## BRIEF SUMMARY OF THE INVENTION

This invention relates to a woven fabric suitable for use in arc protection, the fabric having a first face and a second face, the fabric having a warp yarn dissimilar to a fill yarn, wherein either:

a) a majority of the first face of the fabric is a first yarn that is the warp yarn in the fabric and a majority of the second face of the fabric is a second yarn that is the fill yarn in the fabric; or

b) a majority of the first face of the fabric is a first yarn that is a fill yarn in the fabric and a majority of the second face of the fabric is a second yarn that is the warp yarn in the fabric; and

wherein the second yarn forming the majority of the second face of the fabric comprises:

i) 25 to 100 parts aramid fiber containing 0.5 to 20 weight percent discrete carbon particles, based on the amount of carbon particles in an individual fiber, the carbon particles being homogeneously dispersed in that fiber, and

ii) 0 to 75 parts aramid fiber free of discrete carbon particles; based on the total amount of i) and ii) in the second yarn; and

wherein the first yarn forming the majority of the first face of the article comprises aramid fiber being free of discrete carbon particles;

the fabric having a total content of 0.5 to 3 weight percent discrete carbon particles.

## 2

isophthalamide) (MPD-I) fiber that was free of carbon particles and MPD-I fiber that contained carbon particles, across the entire compositional range (0 to 100%).

FIG. 2 shows the relationship of arc performance versus the total amount of discrete carbon particles in a fabric, normalized for a fabric having a basis weight of 6.3 oz/yd<sup>2</sup>.

DETAILED DESCRIPTION OF THE  
INVENTION

This invention relates to an article of protective clothing comprising woven fabric with a warp-faced or weft-faced twill or satin weave that incorporates a first yarn forming the majority of the outer article surface that comprises aramid fiber being free of discrete carbon particles and a second yarn forming the majority of the inner article surface that comprises 25 to 100 parts aramid fiber containing 0.5 to 20 weight percent discrete carbon particles homogeneously dispersed therein, and 0 to 75 parts aramid fiber free of discrete carbon particles.

The fabric is useful in articles that provided arc protection for workers and other personnel. It has been found that the arc performance of fabrics and garments can be increased on the order of almost two times by the addition of discrete carbon particles in the fire-resistant and thermally stable aramid fiber. As used herein fire-resistant means the polymer has a limiting oxygen index greater than 21 and preferably greater than 25; and the term "thermally stable" means the polymer or fiber retains at least 90 percent of its weight when heated to 425 degrees Celsius at a rate of 10 degrees per minute.

On a fabric weight basis, such dramatic improvement has been found when the total amount of discrete carbon particles in the fabric is 0.5 to 3 weight percent, based on the total amount of fiber in the fabric. FIG. 2 illustrates the ATPV of such a fabric containing carbon particles, normalized for a fabric having a basis weight of 6.3 oz/yd<sup>2</sup>. As illustrated, the presence of carbon can have a significant effect on the fabric arc performance, as measured by ATPV, even at very low loadings. The best performance is found for carbon particles amounts of greater than about 0.5 weight percent in the fabric, with a preferred performance of 12 cal/cm<sup>2</sup> or greater occurring for fabrics having about 0.75 weight percent carbon particles or greater, with an especially desired range being 0.75 to 2 weight percent carbon particles in the fabric.

The two-sided structure of the single-layer fabric allows an outer surface of the fabric, and garments made from the fabric, to be colored (i.e., dyed, etc.) to many different colors including light shades while providing surprisingly improved arc performance. The woven fabric suitable for use in arc protection is a fabric having a first face and a second face, the fabric having a warp yarn dissimilar to a fill yarn, wherein either:

a) a majority of the first face of the fabric is a first yarn that is the warp yarn in the fabric and a majority of the second face of the fabric is a second yarn that is the fill yarn in the fabric; or

b) a majority of the first face of the fabric is a first yarn that is a fill yarn in the fabric and a majority of the second face of the fabric is a second yarn that is the warp yarn in the fabric; and

wherein the second yarn forming the majority of the second face of the article comprises:

i) 25 to 100 parts aramid fiber containing 0.5 to 20 weight percent discrete carbon particles, based on the amount

## BRIEF DESCRIPTION OF THE DRAWINGS

FIG. 1 shows the relationship of the measured lightness value L\* of an intimate blend of natural poly(m-phenylene

of carbon particles in an individual fiber, the carbon particles being homogeneously dispersed in that fiber, and

ii) 0 to 75 parts aramid fiber free of discrete carbon particles; based on the total amount of i) and ii) in the second yarn; and

wherein the first yarn forming the majority of the first face of the fabric comprises aramid fiber being free of discrete carbon particles; the fabric having a total content of 0.5 to 3 weight percent discrete carbon particles. In some embodiments, the aramid fiber in i) is present in an amount of 25 to 50 parts and the aramid fiber in ii) is present in an amount of 50 to 75 parts.

For purposes herein, the term "fiber" is defined as a relatively flexible, macroscopically homogeneous body having a high ratio of length to the width of the cross-sectional area perpendicular to that length. The fiber cross section can be any shape, but is typically round or bean-shaped. Also, such fibers preferably have a generally solid cross section for adequate strength in textile uses; that is, the fibers preferably are not appreciably voided or do not have a large quantity of objectionable voids.

As used herein, the term "staple fibers" refers to fibers that are cut to a desired length or are stretch broken, or fibers that are made having a low ratio of length to the width of the cross-sectional area perpendicular to that length, when compared with continuous filaments. Man-made staple fibers are cut or made to a length suitable for processing on, for example, cotton, woolen, or worsted yarn spinning equipment. The staple fibers can have (a) substantially uniform length, (b) variable or random length, or (c) subsets of the staple fibers have substantially uniform length and the staple fibers in the other subsets have different lengths, with the staple fibers in the subsets mixed together forming a substantially uniform distribution.

In some embodiments, suitable staple fibers have a cut length of from 1 to 30 centimeters (0.39 to 12 inches). In some embodiments, suitable staple fibers have a length of 2.5 to 20 cm (1 to 8 in). In some preferred embodiments the staple fibers made by short staple processes have a cut length of 6 cm (2.4 in) or less. In some preferred embodiments the staple fibers made by short staple processes have a staple fiber length of 1.9 to 5.7 cm (0.75 to 2.25 in) with the fiber lengths of 3.8 to 5.1 cm (1.5 to 2.0 in) being especially preferred. For long staple, worsted, or woolen system spinning, fibers having a length of up to 16.5 cm (6.5 in) are preferred.

The staple fibers can be made by any process. For example, the staple fibers can be cut from continuous straight fibers using a rotary cutter or a guillotine cutter resulting in straight (i.e., non-crimped) staple fiber, or additionally cut from crimped continuous fibers having a saw tooth shaped crimp along the length of the staple fiber, with a crimp (or repeating bend) frequency of preferably no more than 8 crimps per centimeter. Preferably the staple fibers have crimp.

The staple fibers can also be formed by stretch breaking continuous fibers resulting in staple fibers with deformed sections that act as crimps. Stretch broken staple fibers can be made by breaking a tow or a bundle of continuous filaments during a stretch break operation having one or more break zones that are a prescribed distance creating a random variable mass of fibers having an average cut length controlled by break zone adjustment.

Spun staple yarn can be made from staple fibers using traditional long and short staple ring spinning processes that are well known in the art. However, this is not intended to

be limiting to ring spinning because the yarns may also be spun using air jet spinning, open end spinning, and many other types of spinning that converts staple fiber into useable yarns. Spun staple yarns can also be made directly by stretch breaking using stretch-broken tow-to-top staple processes. The staple fibers in the yarns formed by traditional stretch break processes typically have length of up to 18 cm (7 in) long; however, spun staple yarns made by stretch breaking can also have staple fibers having maximum lengths of up to around 50 cm (20 in.) through processes as described for example in PCT Patent Application No. WO 0077283. Stretch broken staple fibers normally do not require crimp because the stretch-breaking process imparts a degree of crimp into the fiber.

Preferably, the yarns in the fabrics are made with a fiber blend. By fiber blend it is meant the combination of two or more staple fiber types in any manner. Preferably the staple fiber blend is an "intimate blend", meaning the various staple fibers in the blend form a relatively uniform mixture of the fibers. In some embodiments the two or more staple fiber types are blended prior to or while the staple fiber yarn is being spun so that the various staple fibers are distributed homogeneously in the staple yarn bundle.

This invention preferably relates to woven fabrics and articles made therefrom that have a warp-faced or weft-faced twill or satin weave. In a twill weave, each weft or filling yarn floats across the warp yarns in a progression of interlacings to the right or left, forming a distinct diagonal line. This diagonal line is also known as a wale. A float is the portion of a yarn that crosses over two or more yarns from the opposite direction. A twill weave requires three or more harnesses, depending on its complexity. Twill weave is often designated as a fraction—such as 2/1—in which the numerator indicates the number of harnesses that are raised (and, thus, threads crossed), in this example, two, and the denominator indicates the number of harnesses that are lowered when a filling yarn is inserted, in this example one. The fraction 2/1 would be read as "two up, one down." The minimum number of harnesses needed to produce a twill weave can be determined by totaling the numbers in the fraction. For the example described, the number of harnesses is three. (The fraction for plain weave is 1/1.) In a satin weave, the fabric surface is almost entirely consists of warp or weft floats since in the repeat of the weave each warp or weft system yarn of passes or floats over or under all but one yarn of the opposite weft or warp system. Generally, the intersection points do not fall in a straight line as in a twill weave but are separated from one another in a regular or irregular formation. One preferred satin weave is a 4/1 weave.

By warp-faced twill or satin weave, it is meant that the quantity of warp yarns is more on the face of the fabric, for example a 2/1 or 3/1 twill. By weft-faced twill or satin weave it is meant the quantity of weft is more on the face of the fabric, for example a 1/2 or 1/3 twill.

The fabric woven with a warp-faced or weft-faced twill or satin weave has warp yarn that is dissimilar to the fill or weft yarn. In a preferred embodiment, the woven fabric has only one type of warp yarn and only one type of fill or weft yarn and the fabric is a single layer fabric.

The fabric forms the inner and outer surface of the article, and because the fabric has a warp-faced or weft-faced twill or satin weave, a majority of the outer surface of the article is a first yarn that is the warp yarn in the fabric and a majority of the inner surface of the article is a second yarn that is the weft or fill yarn in the fabric; or alternatively, a majority of the outer surface of the article is a first yarn that

is the weft or fill yarn in the fabric and a majority of the inner surface of the article is a second yarn that is the warp yarn in the fabric.

The fabric preferably has a first face having a lightness coordinate or "L\*" value of 50 or greater, as measured by the CIELAB color scale. Some embodiments also have a spectral reflectance of 20% or greater over the wavelengths of visible light (380 to 780 nm). The color of fabrics can be measured using a spectrophotometer, also called a colorimeter, which provides three scale values "L\*\*", "a\*\*", and "b\*\*" representing various characteristics of the color of the item measured, and the spectral reflectance. On the color scale, lower "L\*" values generally indicate a darker color, with the color white having a value of about or near 100 and black having a color of about or near 0. In its natural state and before any coloration, poly(meta-phenylene isophthalamide) fiber has a slightly off-white color that when measured using a colorimeter has a "L\*\*" value of about 80 or higher. Poly(meta-phenylene isophthalamide) fiber further comprising 0.5 to 20 weight percent discrete carbon particles has a black color that when measured using a colorimeter has a "L\*\*" value that ranges about 20 or less.

Surprisingly, it has been found that the lightness coordinate or "L\*\*" of a mixture of natural poly(meta-phenylene isophthalamide) fiber, with its slightly off-white color; and poly(meta-phenylene isophthalamide) fiber having carbon particles dispersed therein, with its black color, is not governed by a simple rule of mixtures. FIG. 1 shows the relationship of the measured lightness value L\* of the intimate blend across the entire compositional range (0 to 100%). Blends in the majority of the compositions across the compositional range are actually darker than one would expect by a simple rule of mixtures.

In one embodiment, the second face of the fabric has a "L\*\*" value of 65 or less. In one embodiment, the first face has a "L\*" value of 70 or greater. In some embodiments, the measured color difference between the first face and the second face is at least 5 units on the "L\*\*" scale, and in some preferred embodiments the color difference between the first face and the second face is at least 10 units on the "L\*\*" scale.

As used herein the colors attributed to the fabrics also applies to fibers and fiber blends, yarns, and garments; the same spectrophotometer can be used to determine the "L\*\*" value of fibers, yarns, fabrics, and garments, which generally follow about the same "L\*\*" values.

The woven fabric comprises a first yarn comprising aramid fibers being free of discrete carbon particles and a second yarn comprising aramid fibers, of which at least 25 percent have homogeneously dispersed carbon particles.

Specifically, the second yarn forms a majority of the second face of the fabric and comprises 25 to 100 parts by weight aramid fiber containing 0.5 to 20 weight percent discrete carbon particles, based on the amount of carbon particles in an individual fiber. The carbon particles being homogeneously dispersed in the polymer of that fiber. The second yarn also comprises 0 to 75 parts by weight aramid fiber being free of discrete carbon particles. The aramid fiber is made from an aramid polymer having a Limiting Oxygen Index (LOI) above the concentration of oxygen in air (that is, greater than 21 and preferably greater than 25). This means the fiber or a fabric made solely from that fiber will not support flame and is considered fire-resistant. The aramid fiber also retains at least 90 percent of its weight when heated to 425 degrees Celsius at a rate of 10 degrees per minute, meaning that this fiber has high thermal stability.

It has been found that for the desired arc performance or Arc Thermal Performance Value (ATPV), the carbon-par-

ticle-containing aramid fiber comprises 0.5 to 20 weight percent discrete carbon particles, based on the amount of carbon particles in an individual fiber. In some embodiments, the first staple fiber comprises 0.5 to 10 weight percent discrete carbon particles, based on the amount of carbon particles in an individual fiber; in some embodiments the first staple fiber comprises 0.5 to 6 weight percent discrete carbon particles, based on the amount of carbon particles in an individual fiber. In some other embodiments, it is desirable to have 5 to 10 weight percent discrete carbon particles, based on the amount of carbon particles in an individual fiber. In one preferred embodiment the first staple fiber comprises 0.5 to 3.0 weight percent discrete carbon particles.

As present in the fiber, the carbon particles have an average particle size of 10 micrometers or less, preferably averaging 0.1 to 5 micrometers; in some embodiments an average particle size of 0.5 to 3 micrometers is preferred. In some embodiments an average particle size of 0.1 to 2 micrometers is desirable; and in some embodiments an average particle size of 0.5 to 1.5 micrometers is preferred. Carbon particles include such things as carbon black produced by the incomplete combustion of heavy petroleum products and vegetable oils. Carbon black is a form of paracrystalline carbon that has a higher surface-area-to-volume ratio than soot but lower than that of activated carbon. They are typically incorporated into the fibers by adding the carbon particles to the spin dope prior to the formation of the fibers via spinning.

Essentially any commercially available carbon-black can be used to supply the discrete carbon particles to the aramid polymer composition. They are typically incorporated into the fibers by adding the carbon particles to the spin dope prior to the formation of the fibers via spinning. In one preferred practice, a separate stable dispersion of the carbon-black in a polymer solution, preferably an aramid polymer solution, is first made, and then the dispersion is milled to achieve a uniform particle distribution. This dispersion is the preferably injected into the aramid polymer solution prior to spinning.

The phrase "homogeneously dispersed in that fiber" means that the carbon particles can be found in the fibers uniformly distributed in both the axial and radial directions in the fiber. It is believed that one way of achieving this uniform distribution is by spinning, either by wet or dry spinning, a polymer solution containing the carbon particles.

In some preferred embodiments the polymer used in the aramid fiber is a meta-aramid. As used herein, "aramid" is meant a polyamide wherein at least 85% of the amide (—CONH—) linkages are attached directly to two aromatic rings. Additives can be used with the aramid and, in fact, it has been found that up to as much as 10 percent, by weight, of other polymeric material can be blended with the aramid or that copolymers can be used having as much as 10 percent of other diamine substituted for the diamine of the aramid or as much as 10 percent of other diacid chloride substituted for the diacid chloride of the aramid. Suitable aramid fibers are described in *Man-Made Fibers—Science and Technology*, Volume 2, Section titled *Fiber-Forming Aromatic Polyamides*, page 297, W. Black et al., Interscience Publishers, 1968. Aramid fibers are, also, disclosed in U.S. Pat. Nos. 4,172,938; 3,869,429; 3,819,587; 3,673,143; 3,354,127; and 3,094,511.

Meta-aramid are those aramids where the amide linkages are in the meta-position relative to each other. One preferred meta-aramid is poly(metaphenylene isophthalamide).

Within the yarns, meta-aramid fiber provides a fire resistant fiber with an LOI typically at least about 25.

In some embodiments, the meta-aramid fiber has a minimum degree of crystallinity of at least 20% and more preferably at least 25%. For purposes of illustration, due to ease of formation of the final fiber, a practical upper limit of crystallinity is 50% (although higher percentages are considered suitable). Generally, the crystallinity will be in a range from 25 to 40%. The degree of crystallinity of a meta-aramid fiber can be determined by one of two methods. The first method is employed with a non-voided fiber while the second is employed on a fiber that is not totally free of voids. The percent crystallinity of meta-aramids in the first method is determined by first generating a linear calibration curve for crystallinity using good, essentially non-voided samples. For such non-voided samples the specific volume (1/density) can be directly related to crystallinity using a two-phase model. The density of the sample is measured in a density gradient column. A meta-aramid film, determined to be non-crystalline by x-ray scattering methods, was measured and found to have an average density of 1.3356 g/cm<sup>3</sup>. The density of a completely crystalline meta-aramid sample was then determined from the dimensions of the x-ray unit cell to be 1.4699 g/cm<sup>3</sup>. Once these 0% and 100% crystallinity end points are established, the crystallinity of any non-voided experimental sample for which the density is known can be determined from this linear relationship:

$$\text{Crystallinity} = \frac{(1/\text{non-crystalline density}) - (1/\text{experimental density})}{(1/\text{non-crystalline density}) - (1/\text{fully crystalline density})}$$

Since many fiber samples are not totally free of voids, Raman spectroscopy is the preferred method to determine crystallinity. Since the Raman measurement is not sensitive to void content, the relative intensity of the carbonyl stretch at 1650-1 cm can be used to determine the crystallinity of a meta-aramid in any form, whether voided or not. To accomplish this, a linear relationship between crystallinity and the intensity of the carbonyl stretch at 1650 cm<sup>-1</sup>, normalized to the intensity of the ring stretching mode at 1002 cm<sup>-1</sup>, was developed using minimally voided samples whose crystallinity was previously determined and known from density measurements as described above. The following empirical relationship, which is dependent on the density calibration curve, was developed for percent crystallinity using a Nicolet Model 910 FT-Raman Spectrometer:

$$\% \text{ Crystallinity} = \frac{100.0 \times (I(1650 \text{ cm}^{-1}) - 0.2601)}{0.1247}$$

where  $I(1650 \text{ cm}^{-1})$  is the Raman intensity of the meta-aramid sample at that point. Using this intensity, the percent crystallinity of the experiment sample is calculated from the equation.

Meta-aramid fibers, when spun from solution, quenched, and dried using temperatures below the glass transition temperature, without additional heat or chemical treatment, develop only minor levels of crystallinity. Such fibers have a percent crystallinity of less than 15 percent when the crystallinity of the fiber is measured using Raman scattering techniques. These fibers with a low degree of crystallinity are considered amorphous meta-aramid fibers that can be crystallized through the use of heat or chemical means. The

level of crystallinity can be increased by heat treatment at or above the glass transition temperature of the polymer. Such heat is typically applied by contacting the fiber with heated rolls under tension for a time sufficient to impart the desired amount of crystallinity to the fiber.

The level of crystallinity of m-aramid fibers can also be increased by a chemical treatment, and in some embodiments this includes methods that color, dye, or mock dye the fibers prior to being incorporated into a fabric. Some methods are disclosed in, for example, U.S. Pat. Nos. 4,668,234; 4,755,335; 4,883,496; and 5,096,459. A dye assist agent, also known as a dye carrier may be used to help increase dye pick up of the aramid fibers. Useful dye carriers include aryl ether, benzyl alcohol, or acetophenone.

The first yarn forms the majority of the other face of the fabric that is preferably used as the outer surface of a garment made from the fabric. The first yarn comprises aramid fiber being free of discrete carbon particles, meaning that the fiber does not contain carbon particles as defined herein. In one embodiment, the aramid fiber being free of discrete carbon particles is further capable of accepting a dye or coloration. Other fibers can be mixed with the aramid fiber in the first yarn. In a preferred embodiment, the aramid fiber being free of discrete carbon particles is present as a majority fiber (greater than 50 weight percent) in the first yarn, and some embodiments the aramid fiber is present as a staple fiber or a blend of aramid fibers with or without other fibers.

In some preferred embodiments, the aramid fiber being free of discrete carbon particles in the first yarn is a meta-aramid fiber as previously described herein. One preferred meta-aramid is poly(metaphenylene isophthalamide). In some embodiments, the meta-aramid fiber has a minimum degree of crystallinity of at least 20% and more preferably at least 25%. For purposes of illustration, due to ease of formation of the final fiber, a practical upper limit of crystallinity is 50% (although higher percentages are considered suitable). Generally, the crystallinity will be in a range from 25 to 40%.

In some embodiments, the meta-aramid fiber used in either the first or second yarns can have an axial thermal shrinkage at 185 degrees Celsius of greater than 10 percent. This high level of shrinkage is representative of an amorphous fiber that has not been appreciably crystallized or otherwise heat stabilized. Representative meta-aramid fibers have a percent crystallinity of less than 15 percent when the crystallinity of the fiber is measured using Raman scattering techniques. Due to the lack of crystallinity, such fibers can be relatively easily dyed, either in intimate blend, yarn, fabric, or article form. One preferred meta-aramid is poly(metaphenylene isophthalamide).

In some embodiments, the meta-aramid fiber used in either the first or second yarns can have an axial thermal shrinkage at 185 degrees Celsius of 2 percent or less. This low level of shrinkage is representative of a relatively crystallized fiber. Representative meta-aramid fibers have a minimum degree of crystallinity of at least 20% and more preferably at least 25%. For purposes of illustration, due to ease of formation of the final fiber, a practical upper limit of crystallinity is 50% (although higher percentages are considered suitable). Generally, the crystallinity will be in a range from 25 to 40%. Due to this crystallinity, such fibers can be dyed, either in intimate blend, yarn, fabric, or article form, but generally require dye assists or more aggressive dyeing conditions. One preferred meta-aramid is poly(metaphenylene isophthalamide).

In some embodiments, the aramid fiber being free of discrete carbon particles further comprises a dye. Suitable dyes preferably provide colors that have an "L\*\*" value of 40 or greater, preferably 50 or greater. One preferred range of "L\*\*" values is from 50 to 90.

In some embodiments, the first and/or second yarns can further comprise para-aramid fibers, and the preferred para-aramid is poly(paraphenylene terephthalamide), preferably used in an amount that is up to about 8 percent by weight in the yarns. In some embodiments, the first and/or second yarns can further comprise a very minor amount (1-3% by weight of the yarn) of an antistat fiber, one suitable antistat fiber is melt-spun thermoplastic antistatic fibers such as those described in U.S. Pat. No. 4,612,150 to De Howitt and/or U.S. Pat. No. 3,803,453 to Hull. These fibers, while they contain carbon black, have a negligible impact on arc performance, since the fiber polymer does not have the combination of being flame resistant and thermally stable; that is, it does not have in combination a LOI of greater than 21, preferably greater than 25, and does not retain at least 90 percent of its weight when heated to 425 degrees Celsius at a rate of 10 degrees per minute. In fact, such thermoplastic antistat fibers lose in excess of 35 weight percent when heated to 425 degrees Celsius at a rate of 10 degrees per minute. For the purposes herein, and to avoid any confusion, the total content in the weight percent of discrete carbon particles is based on the total weight of the fiber blend, excluding any minor amount of antistat fibers.

In one preferred embodiment, the first and second yarns are spun staple yarns made from an intimate blend of staple fibers. The intimate blend of staple fibers can be made by cutter blending strands or tows of different fibers or by blending different bales of fibers and other means known in the art of forming an intimate blend. For example, the two or more slivers of different staple fiber types can be blended prior to or while a staple fiber yarn is being spun so that the various staple fibers are distributed homogeneously as an intimate blend in the staple yarn bundle.

By "yarn" is meant an assemblage of fibers spun or twisted together to form a continuous strand. As used herein, a yarn generally refers to what is known in the art as a singles yarn, which is the simplest strand of textile material suitable for such operations as weaving and knitting; or a ply yarn or plied yarn. A spun staple yarn can be formed from staple fibers with more or less twist. When twist is present in a singles yarn, it is all in the same direction. As used herein the phrases "ply yarn" and "plied yarn" can be used interchangeably and refer to two or more yarns, i.e. singles yarns, twisted or plied together.

In some particularly useful embodiments, the fabrics described herein can be used to make arc- and flame-resistant garments. In some embodiments the garments can have essentially one layer of the protective fabric. Garments of this type include jumpsuits, coveralls, pants, shirts, gloves, sleeves and the like that can be worn in situations such as chemical processing industries or industrial or electrical utilities where an extreme thermal event might occur. Preferably, the outer surface of the garment, the surface closer to the potential electrical arc, comprises a majority of the yarns comprising the aramid fiber free of carbon particles, and the inner surface of the garment, the surface closer to the wearer, comprises a majority of the yarns comprising the aramid fiber containing carbon particles. In some embodiments the woven fabric contains a first yarn that further comprises a dye. In this manner, the outer surface of the garment can be colored, dyed, or printed

with a dye to have any number of colors and shades and is not limited to a dark or black color.

Protective articles or garments of this type include protective coats, jackets, jumpsuits, coveralls, hoods, etc. used by industrial personnel such as electricians and process control specialists and others that may work in an electrical arc potential environment. In a preferred embodiment, the protective garment is a coat or jacket, including a three-quarter length coat commonly used over the clothes and other protective gear when work on an electrical panel or substation is required.

In a preferred embodiment, the protective articles or garments have at least a Category 1 or 2 arc rating or higher as measured by either of two common category rating systems for arc ratings. The National Fire Protection Association (NFPA) has 4 different categories with Category 1 having the lowest performance and Category 4 having the highest performance. Under the NFPA 70E system, Categories 1, 2, 3, and 4 correspond to a heat flux through the fabric of 4, 8, 25, and 40 calories per square centimeter, respectively. The National Electric Safety Code (NESC) also has a rating system with 3 different categories with Category 1 having the lowest performance and Category 3 having the highest performance. Under the NESC system, Categories 1, 2, and 3 correspond to a heat flux through the fabric of 4, 8, and 12 calories per square centimeter, respectively. Therefore, a fabric or garment having a Category 2 arc rating can withstand a thermal flux of 8 calories per square centimeter, as measured per standard set method ASTM F1959 or NFPA 70E.

#### Test Methods

**Arc Resistance.** The arc resistance of fabrics of this invention is determined in accordance with ASTM F-1959-99 "Standard Test Method for Determining the Arc Thermal Performance Value of Materials for Clothing". Preferably fabrics of this invention have an arc resistance (ATPV) of at least 0.8 calories and more preferably at least 2 calories per square centimeter per ounce per square yard.

**ThermoGravimetric Analysis (TGA).** Fiber that retains at least 90 percent of its weight when heated to 425 degrees Celsius at a rate of 10 degrees per minute can be determined using a Model 2950 Thermogravimetric Analyzer (TGA) available from TA Instruments (a division of Waters Corporation) of Newark, Del. The TGA gives a scan of sample weight loss versus increasing temperature. Using the TA Universal Analysis program, percent weight loss can be measured at any recorded temperature. The program profile consists of equilibrating the sample at 50 degrees C.; ramping the temperature 10° C. per minute from 50 to 1000 degrees C.; using air as the gas, supplied at 10 ml/minute; and using a 500 microliter ceramic cup (PN 952018.910) sample container. A specific testing procedure is as follows. The TGA was programmed using the TGA screen on the TA Systems 2900 Controller. The sample ID was entered and the planned temperature ramp program of 20 degrees per minute selected. The empty sample cup was tared using the tare function of the instrument. The fiber sample was cut into approximately  $\frac{1}{16}$ " (0.16 cm) lengths and the sample pan was loosely filled with the sample. The sample weight should be in the range of 10 to 50 mg. The TGA has a balance therefore the exact weight does not have to be determined beforehand. None of the sample should be outside the pan. The filled sample pan was loaded onto the balance wire making sure the thermocouple is close to the top edge of the pan but not touching it. The furnace is raised

## 11

over the pan and the TGA is started. Once the program is complete, the TGA will automatically lower the furnace, remove the sample pan, and go into a cool down mode. The TA Systems 2900 Universal Analysis program is then used to analyze and produce the TGA scan for percent weight loss over the range of temperatures.

Limited Oxygen Index. The limited oxygen index (LOI) of fabrics of this invention is determined in accordance with ASTM G-125-00 "Standard Test Method for Measuring Liquid and Solid Material Fire Limits in Gaseous Oxidants".

Color Measurement. The system used for measuring color and spectral reflectance is the 1976 CIELAB color scale ( $L^*a^*b^*$  system developed by the Commission Internationale de l'Eclairage). In the CIE " $L^*a^*b^*$ " system, color is viewed as point in three-dimensional space. The " $L^*$ " value is the lightness coordinate with high values being the lightest, the " $a^*$ " value is the red/green coordinate with " $+a^*$ " indicating red hue and " $-a^*$ " indicating green hue and the " $b^*$ " value is the yellow/blue coordinate with " $+b^*$ " indicating yellow hue and " $-b^*$ " indicating blue hue. A spectrophotometer was used to measure the color of samples, either in puffs of fiber or in fabric or garment form as indicated. Specifically, a Hunter Lab UltraScan® PRO spectrophotometer was used, including the industry standard of 10-degree observer and D65 illuminant. The color scale used herein uses the coordinates of the CIE (" $L^*a^*b^*$ ") color scale with the asterisk, as opposed to the coordinates of the older Hunter color scale, which are designated (" $L-a-b$ ") without the asterisk.

Weight Percent of Carbon Particles. The nominal amount of carbon black in the fiber, when making the fiber, is determined by a simple mass balance of ingredients. After the fiber is made, the amount of carbon black present in the fiber can be determined by measuring the weight of a sample of fiber, removing the fiber by dissolution of the polymer in a suitable solvent that does not affect the carbon black particles, washing the remaining solids to remove any inorganic salts that are not carbon, and weighing the remaining solids. One specific method includes weighing about a gram of the fiber, yarn, or fabric to be tested and heating that sample in an oven at 105° C. for 60 minutes to remove any moisture, followed by placing the sample in a desiccator to cool to room temperature, followed by weighing the sample to obtain an initial weight to a precision of 0.0001 grams. The sample is then placed in a 250 ml flat bottom flask with a stirrer and 150 ml of a suitable solvent, for example 96% sulfuric acid, is added. The flask is then placed on a combination stir/heater with a chilled water condenser operating with enough flow to prevent any fumes from exiting the top of the condenser. The heat is then applied while stirring until the yarn is fully dissolved in the solvent. The flask is then removed from the heater and allowed to cool to room temperature. The contents of the flask are then vacuum filtered using a Millipore vacuum filter unit with a tared 0.2 micron PTFE filter paper. Remove the vacuum and then rinse the flask out with 25 ml of additional solvent, which is also passed through the filter. The Millipore unit is then removed from the vacuum flask and reset on a new clean glass vacuum flask. With vacuum, the residue on the filter paper is washed with water until a pH paper check on the filtrate indicates the wash water to be neutral. The residue is then finally washed with methanol. The filter paper with residue sample is removed, placed in a dish, and heated in an oven at 105° C. to dry for 20 minutes. The filter paper with residue sample is then put in a desiccator to cool to room temperature, followed by weighing the filter paper with residue sample to obtain the final weight to a precision

## 12

of 0.0001 grams. The weight of the filter is subtracted from the weight of the filter paper with residue sample. This weight is then divided by the initial weight of the yarn or fiber or fabric and multiplied by 100. This will give the weight percentage of the carbon black in the fiber, yarn, or fabric.

Particle Size. Carbon particle size can be measured using the general provisions of ASTM B822-10—"Standard Test Method for Particle Size Distribution of Metal Powders and Related Compounds by Light Scattering".

Shrinkage. To test for fiber shrinkage at elevated temperatures, the two ends of a sample of multi-filament yarn to be tested are tied together with a tight knot such that the total interior length of the loop is approximately 1 meter in length. The loop is then tensioned until taut and the doubled length of the loop measured to the nearest 0.1 cm. The loop of yarn is then hung in an oven for 30 minutes at 185 degrees Celsius. The loop of yarn is then allowed to cool, it is re-tensioned and the doubled length is re-measured. Percent shrinkage is then calculated from the change in the linear length of the loop.

## Examples

In the examples that follow, unless designated differently, the natural meta-aramid fiber was amorphous or uncrosslinked poly(m-phenylene isophthalamide) (MPD-I) fiber, and the natural para-aramid fiber was poly(p-phenylene terephthalamide) (PPD-T); both of these were free of carbon particles, that is, they did not contain any added carbon-black. The black meta-aramid fiber was crystallized MPD-I fiber that further contained carbon particles or carbon-black. The antistatic fiber was a carbon-core nylon-sheath fiber known commercially as P140® available from Invista.

The calculated percent total amount of carbon (percent) for the intimate blend (and in the fabric) was based on the weight of the carbon particles in the carbon-containing black meta-aramid fiber, which had a nominal 2.1 weight percent carbon, divided by the weight of the total fiber blend, times 100. Any carbon in the antistatic fiber is not considered in the calculation of percent carbon in the blend.

## Reference Example

To illustrate the effect the carbon containing fiber has on the lightness of fabrics, intimate blends of natural poly(m-phenylene isophthalamide) (MPD-I) fiber that was free of carbon particles and MPD-I fiber that contained carbon particles (black fiber) were made across the entire compositional range (0 to 100%). The compositions are shown in Table 1. Each blend was carded to create a "puff" ball of fibers for lightness measurement. The  $L^*$  value for each blend was measured using a HunterLab UltraScan® PRO spectrophotometer with the following viewing conditions: Large Area View/10-degree observer/D65 illuminant. The color scale used for reporting  $L^*$  values is the CIE 1976  $L^*a^*b^*$  (CIELAB) color scale. A low value on this scale indicates a dark shade, while a high value indicates a light shade. As summarized in Table 2, the  $L^*$  value increases with decreasing amounts of the black MPD-I fiber.

FIG. 1 shows the relationship of the measured lightness value  $L^*$  graphically across the entire compositional range, illustrating that surprisingly the lightness of the blends is not governed by a simple rule of mixtures.

TABLE 1

| Percent Black Fiber | Percent Natural Fiber | L* Value | a* Value | b* Value |
|---------------------|-----------------------|----------|----------|----------|
| 0                   | 100                   | 96       | -0.30    | 2.85     |
| 3                   | 97                    | 80       | -0.04    | 0.45     |
| 5                   | 95                    | 76       | 0.04     | 0.21     |
| 10                  | 90                    | 67       | 0.1      | -0.11    |
| 15                  | 85                    | 62       | 0.05     | -0.38    |
| 25                  | 75                    | 54       | 0.12     | -0.47    |
| 35                  | 65                    | 48       | 0.11     | -0.61    |
| 50                  | 50                    | 39       | 0.12     | -0.65    |
| 75                  | 25                    | 29       | 0.08     | -0.92    |
| 100                 | 0                     | 20       | 0.02     | -1.1     |

## Example 1

A durable arc and thermal protective woven fabric, having an outer surface having a lighter color than the inner surface was prepared having different warp and fill air-jet spun yarns.

The warp yarn was made from an intimate staple fiber blend of 93 weight percent natural meta-aramid fiber, 5 weight percent natural para-aramid fiber, and 2 weight percent antistatic fiber. A picker blend sliver of the meta-aramid fiber, para-aramid fiber, and antistatic fiber was prepared and was made into spun staple yarn using cotton system processing and an airjet spinning frame. The resultant yarn was a 21 tex (28 cotton count) single yarn. Two single yarns were then plied on a plying machine to make a two-ply yarn having a ply twist of 10 turns/inch twist. This plied yarn was used as the warp yarn.

The fill yarn was made from an intimate staple fiber blend of 50 weight percent of a first fiber blend, which consisted of 93 weight percent natural meta-aramid fiber, 5 weight percent natural para-aramid fiber, and 2 weight percent antistatic fiber; combined with 50 weight percent of a second fiber blend that consisted of 95 weight percent black meta-aramid fiber provided with approximately 2 weight percent homogeneously dispersed carbon particles and 5 weight percent natural para-aramid fiber. A picker blend sliver of the first and second fiber blends were made into a spun staple yarn using cotton system processing and an airjet spinning frame. The resultant yarn was a 21 tex (28 cotton count) single yarn. Two single yarns were then plied on a plying machine to make a two-ply yarn having a ply twist of 10 turns/inch twist. This plied yarn was used as the fill yarn.

The yarns were then used as in the warp and fill of a fabric that was woven on a shuttle loom in a warp-faced 2×1 twill construction. The greige twill fabric had a basis weight of 186 g/m<sup>2</sup> (5.5 oz/yd<sup>2</sup>). The greige twill fabric was then scoured in hot water and was mock dyed using a dye carrier/assist (Cindye C-45) but no dye and dried. The L\* value for each side was measured using a HunterLab Ultra-Scan® PRO spectrophotometer. The results are shown in Table 2.

The finished twill fabric had a construction of approximately 31 ends×16 picks per cm (77 ends×47 picks per inch) and a basis weight of 203 g/m<sup>2</sup> (6.0 oz/yd<sup>2</sup>). The final fabric has a total carbon particle concentration from the aramid fiber of 0.4 weight percent.

The finished fabric was then tested to determine its Arc Thermal Performance Value (ATPV). This was compared to a control fabric constructed in a similar manner, which was a standard aramid fabric comprising identical warp and fill yarns, each made from an intimate staple fiber blend of 93

weight percent natural meta-aramid fiber, 5 weight percent natural para-aramid fiber, and 2 weight percent antistatic fiber. The results are shown in the Table 2.

As shown, the final fabric had a dramatic increase in arc performance while providing at least one surface that did not show an objectionable level of the carbon-containing fiber and which could be dyed various colors.

TABLE 2

| Item    | Basis Weight,<br>oz/yd <sup>2</sup><br>(g/m <sup>2</sup> ) | L* Value,<br>1 <sup>st</sup> Side | L* Value,<br>2 <sup>nd</sup> Side | ATPV,<br>cal/cm <sup>2</sup> |
|---------|------------------------------------------------------------|-----------------------------------|-----------------------------------|------------------------------|
| Control | 6.0<br>(203)                                               | 84                                | 84                                | 6.5                          |
| Example | 6.0<br>(203)                                               | 73                                | 61                                | 8.9                          |

## Example 2

Additional samples of the greige twill fabric made in Example 1 were further dyed using a pressure jet dyeing vessel into which the fabric is loaded and then circulated through an apertured venturi in a continuous loop achieved by sewing the ends of the fabric together. The fabric was scoured for 10 minutes at a temperature of 60 degrees Celsius in an aqueous solution. After scouring the dyeing vessel was drained and charged with dye, dye assistant ((Cindye C-45), and water at an initial temperature of 70 degrees Celsius. The fabric was dyed for 10 minutes while the bath temperature was increased at a rate of 1 degree Celsius per minute. The pH of the solution was then adjusted by the addition of acetic acid to a pH of between 3 and 4. The vessel was then charged with additional dye and dye assistant and a constant temperature of 80 degrees Celsius was maintained for 10 minutes. The temperature was then raised as a rate of 1 degree Celsius per minute until the bath temperature is 130 degrees Celsius. The bath was maintained at 130 degrees Celsius for 40 minutes or until the dye was exhausted. The bath was then cooled to 60 degrees Celsius and drained. The vessel was then charged with a solution of 2 grams per liter sodium hydrosulfite, 2 grams per liter sodium carbonate, and water to neutralize the dye solution. The bath temperature was raised at a rate of 1 degree Celsius per minute to 60 degrees Celsius and allowed to circulate for 10 minutes. The vessel was then drained and recharged with water. The water temperature was then raised at a rate of 1 degree Celsius per minute to a temperature of 60 degrees Celsius and allowed to circulate for 10 minutes. The vessel was then drained and the fabric dried.

The above process was used multiple times with red, teal, royal blue, navy blue, and khaki dyes to make red, teal, royal blue, navy blue, and khaki dyed two-side fabrics. The resulting dyed fabric had a face side dyed with a desirable shade of the color, with the other side having a slightly darker color, due to the higher percentage of the carbon containing fiber on that side.

What is claimed is:

1. A woven fabric suitable for use in arc protection, the fabric having a first face and a second face, the fabric having a warp yarn dissimilar to a fill yarn, wherein either:
  - a majority of the first face of the fabric is a first yarn that is the warp yarn in the fabric and a majority of the second face of the fabric is a second yarn that is the fill yarn in the fabric; or

**15**

- b) a majority of the first face of the fabric is a first yarn that is a fill yarn in the fabric and a majority of the second face of the fabric is a second yarn that is the warp yarn in the fabric; and  
 wherein the second yarn forming the majority of the second face of the fabric comprises:  
 i) 25 to 100 parts aramid fiber containing 0.5 to 20 weight percent discrete carbon particles, based on the amount of carbon particles in an individual fiber, the carbon particles being homogeneously dispersed in that fiber, and  
 ii) 0 to 75 parts aramid fiber free of discrete carbon particles; based on the total amount of i) and ii) in the second yarn; and  
 wherein the first yarn forming the majority of the first face of the fabric comprises aramid fiber being free of discrete carbon particles;  
 the fabric having a total content of 0.5 to 3 weight percent discrete carbon particles.
2. The woven fabric of claim 1 wherein the aramid fiber in i) is present in an amount of 25 to 50 parts, and the aramid fiber in ii) is present in an amount of 50 to 75 parts.
3. The woven fabric of claim 1 wherein the aramid fiber in i) comprises 0.5 to 6 weight percent discrete carbon particles.

5

10

15

**16**

4. The woven fabric of claim 1 wherein the aramid fiber in i) is a meta-aramid.
5. The woven fabric of claim 4 wherein the meta-aramid is poly(meta-phenylene isophthalamide).
6. The woven fabric of claim 1 wherein the aramid fiber in ii) is a meta-aramid or a para-aramid.
7. The woven fabric of claim 6 wherein the meta-aramid is poly(meta-phenylene isophthalamide) and the para-aramid is poly(para-phenylene terephthalamide).
8. The woven fabric of claim 1 wherein the first yarn and the second yarn comprise staple fibers.
9. The woven fabric of claim 1 wherein the second yarn comprises an intimate blend of staple fibers.
10. The woven fabric of claim 1 wherein the first yarn further comprises a dye.
11. An article of thermal protective clothing comprising the woven fabric of claim 1.
12. The article of thermal protective clothing of claim 11 wherein the woven fabric is positioned in the clothing such that the first face of the woven fabric is closer to a potential arc event than the second face of the fabric.

\* \* \* \* \*